

Jan. 27, 1931.

G. T. MAHLER ET AL

1,790,012

CONDENSING METALLIC VAPORS

Filed May 5, 1925

2 Sheets-Sheet 1

Fig. 1



Fig. 2



Fig. 3



INVENTORS  
George T. Mahler  
Ernest C. Handwerk  
BY Earl H. Bance  
Pennie, Danis, Marin, Edmonds  
ATTORNEYS

Jan. 27, 1931.

G. T. MAHLER ET AL  
CONDENSING METALLIC VAPORS

1,790,012

Filed May 5, 1925

2 Sheets-Sheet 2



INVENTORS  
George T. Mahler  
Erwin C. Handwerk  
BY Carl H. Bunc  
Pennie, Davis, Marvin & Edmonds  
ATTORNEYS

## UNITED STATES PATENT OFFICE

GEORGE T. MAHLER, ERWIN C. HANDWERK, AND EARL H. BUNCE, OF PALMERTON, PENNSYLVANIA, ASSIGNORS TO THE NEW JERSEY ZINC COMPANY, OF NEW YORK, N. Y., A CORPORATION OF NEW JERSEY

## CONDENSING METALLIC VAPORS

Application filed May 5, 1925. Serial No. 28,056.

This invention relates to the condensation of metallic vapor, and more particularly zinc vapor, and has for its object the provision of an improved method of and apparatus for condensing metallic vapor and especially zinc vapor.

Metallic zinc or spelter, when produced by the reduction of oxidized zinc ores at high temperatures, is almost universally made at the present time in zinc distillation or spelter furnaces having a number of relatively small retorts to the outer ends of which condensers are attached. The retorts are usually mounted at a slight inclination, 15 usually inclined downward from the butt or closed end towards the open or outer end. The condenser is in effect an extension or elongation of the retort, although usually mounted in a substantially horizontal position, and hence not in exact alignment with the elongated axis of the retort. The zinc vapor and other gases pass in a substantially horizontal line from the retort through the condenser, and the exhaust gases escape through the open end of the condenser. The efficiency of this present customary condensing apparatus is far from satisfactory, only about 60 to 65% of the metallic zinc vapor passing out of the retort 20 being condensed as metallic zinc or spelter, the remainder being condensed as "blue powder" or burning at the mouth of the condenser to zinc oxide and lost.

We have discovered that the efficiency of condensation of zinc vapor can be very substantially improved by appropriately circulating the vapor over a film of molten zinc of suitable area and held at a carefully controlled temperature. The necessary film of molten zinc is preferably provided and maintained upon the ceiling and the upright wall or walls of the condensing chamber, and the zinc vapor entering the chamber is caused to repeatedly circulate and contact 40 with the film of molten zinc. The desired circulation of the zinc vapor is advantageously brought about by passing a stream or current of zinc vapor into the condensing chamber and causing this stream of vapor to 45 impinge against a ceiling so disposed as to

uniformly deflect the zinc vapor against the film of molten zinc on the ceiling and upright wall or walls of the condensing chamber.

In our preferred practice, the condensing 55 chamber is disposed so that the stream of zinc vapor passes upwardly through the bottom thereof and impinging against the ceiling is uniformly deflected outwardly and downwardly over the film of molten zinc on 60 the ceiling and the upright (preferably vertical) wall or walls of the condensing chamber. The zinc vapor is thus caused to repeatedly circulate over and in contact with the film of molten zinc, of appropriate area, 65 and at the proper temperature, and condenses thereon. The condensed zinc serves to maintain on the ceiling and on the upright wall or walls of the condensing chamber the desired film of molten zinc, and the excess zinc 70 drops off or flows down these walls to an appropriate well at the bottom of the condensing chamber and is there collected.

We have found that in addition to the area of the condensing surface careful control of the temperature of the ceiling and upright wall or walls of the condensing chamber is necessary for the optimum efficiency of condensation of the zinc vapor. When the temperature of the ceiling and upright wall (or walls) is properly controlled 75 substantially all of the zinc vapor is condensed as metallic zinc or liquid spelter, and less than 10% and frequently as little as 1 to 2% of the total zinc entering the chamber 80 condenses as "blue powder" or uncoalesced zinc droplets, the balance of the zinc being condensed as metallic zinc or liquid spelter.

In the accompanying drawings, we have 85 illustrated what we now consider the best modes of practicing the invention. In these drawings, we have shown our improved condenser in conjunction with a vertical retort or shaft furnace, but we desire to have it understood that the invention is not limited to this particular type of zinc distillation furnace but, on the contrary, the invention is of 90 general applicability and can be advantageously used for condensing zinc or other me- 95 100

talic vapor without regard to the source of the vapor.

In the accompanying drawings

Fig. 1 is a front sectional elevation of a vertical retort or shaft furnace for reducing oxidized zinc ores provided with the improved condenser of the invention for condensing the metallic zinc vapors;

Fig. 2 is a side sectional elevation of the same apparatus;

Fig. 3 is a section on the line 3—3 of Fig. 2; and

Figs. 4, 5, 6, 7, 8 and 9 are sectional elevations of various modified forms of condensers embodying the principles of our invention.

The zinc distillation furnace illustrated in Figs. 1, 2 and 3 of the drawings comprises a vertical retort 10 of fire-clay or other appropriate material. The retort 10 is surrounded, for the greater part of its length, by a laboratory or heating chamber 11. The heating chamber 11 is built within a furnace structure comprising an outer steel shell or casing 12, an intermediate layer 13 of heat-insulating material, such as Sil-o-cel, and a lining made up of fire-brick 14 covered with graphite blocks or plates 15. Appropriate openings 16 are provided through the wall of the furnace structure for permitting the insertion of pyrometers within the laboratory or heating chamber 11, for ascertaining and controlling the temperature throughout the length of this chamber.

The furnace structure is mounted on an appropriate foundation 17. The bottom of the retort 10 opens into a closed chamber or pit 18 having a clean-out door 19.

Any appropriate means may, of course, be employed for heating the retort 10. Thus, for example, fire gases may be conducted through the laboratory 11 and around the retort 10. In the apparatus illustrated in Figs. 1, 2 and 3, the heating of the retort is effected by electric energy. The electric heating or resistance element comprises two graphite rods 20 extending through the top of the furnace structure and resting on graphite blocks 21 slightly below the center of the chamber 11. The lower portion of the rods 20 are hollow and have a spiral slot so as to provide a helical resistance path for the flow of the electric current. One terminal of the source of electric energy is connected to one of the graphite rods 20 and the other terminal of the source of electric energy is connected to the other graphite rod 20, the electric circuit between the lower ends of the two rods 20 being completed through the graphite blocks 21 and the graphite lining 15. Either direct or alternating current may be used for supplying electric energy to the graphite rods 20.

The bottom of the chamber 11 is provided with two graphite resistance rods or elements

22, of the same general construction as the rods 20. The rods 22 rest on graphite blocks 23 which serve to electrically connect in parallel the intermediate portions of the two rods. This lower heating element may often be disposed with, and is provided as an auxiliary or additional source of heat when desired or necessary.

The improved condenser of our invention is vertically mounted on top of the furnace structure and axially in alignment with the retort 10. In Figs. 1 and 2 of the drawings, this condenser comprises a cylindrical, vertically disposed wall 25. A flat, circular ceiling 26 covers the top of the cylinder 25, and an annular plate 27 partially closes the bottom of the cylinder. The cylinder 25 and plates 26 and 27 are made of heat refractory material, such as fire clay, carborundum, mixtures of the same, or the like. These three elements may be integrally united or separately formed and joined together to constitute the novel and improved "plug-hat" condenser of our invention.

A nozzle 28 is attached to the bottom plate 27. The diameter of the central opening in the plate 27 and the internal diameter of the nozzle 28 are less than the diameter of the retort 10 and these three elements are axially in alignment. The nozzle 28 extends upwardly to about midway of the condensing chamber provided within the cylinder 25.

The ceiling 26 has a central opening 30 loosely covered by a plate 31. The exterior of the condenser (cylinder 25 and ceiling 26) is covered with an appropriate layer 29 of heat insulating material. In practice, we have found dust coal admirably adapted as the heat insulating covering for the condenser. From the loosely packed insulating material (coal) around the plate 31, the carbon monoxide gas escapes from the opening 30 of the condensing chamber and burns in the air.

The annular space between the nozzle 28 and the cylinder 25 provides a well for collecting molten zinc, and molten zinc is tapped from this well, from time to time, through a tap-hole 32.

The mixture of zinc vapor and carbon monoxide gas (resulting from the reduction of the oxidized zinc ore in the retort 10) passes out of the top of the retort into the nozzle 28. An upwardly flowing stream or current of zinc vapor thus passes through the bottom of the condenser and into the condensing chamber. This stream of zinc vapor impinges against the fans out over the ceiling 26, and is uniformly deflected down the side of the upright wall 25, as indicated by the arrows in Fig. 1 of the drawings.

The inner surface of the cylindrical wall 25 and the entire ceiling 26 are covered with a film of molten zinc (indicated by the line a). The zinc vapors entering the condenser are

drafted across this constantly renewed fresh film of molten zinc and condense thereon. Thus, the film of molten zinc provides a nucleus upon which condensation of the zinc vapor readily takes place. The exhaust gases, for the most part carbon monoxide, escape through the opening 30, passing underneath the loose plate 31 and through the loose heat insulating material thereon.

10 By properly regulating the temperature of the condensing walls (25 and 26) substantially all of the zinc vapor will condense as metallic zinc or liquid spelter.

The metallic zinc condensing on the wall 15 of the cylinder 25 flows down this wall into the molten metal well at the bottom of the condensing chamber. The molten zinc accumulates in this well and is periodically removed therefrom through the tap-hole 32.

20 The film of molten zinc on the condensing walls need not be continuous, and in practice may consist of minute drops or globules of molten zinc which substantially cover the inner surface of the wall or walls. By a film 25 of molten zinc, we mean a thin layer of molten zinc, not necessarily continuous, but sufficiently extensive in area to substantially cover the inner or condensing surface of the cylinder 25 and ceiling 26.

30 It is important that the temperature of the walls of the condensing chamber (25 and 26) be carefully controlled. If the temperature of these walls is too high, the gases escaping through the opening 30 will carry too much 35 zinc vapor, and if the temperature of these walls is too low an excessive amount of "blue powder" will be formed. We have found a temperature of from 500 to 850° C. satisfactory, and when the condensing walls are maintained within this temperature range, 40 very efficient condensation of the zinc vapor to metallic zinc or liquid spelter results.

We prefer to regulate and control the temperature of the condensing wall or walls by 45 regulating the amount of external heat insulation on these walls. In practice, we periodically insert a pyrometer (thermo-couple) into the condensing chamber (preferably through the top opening 30) and when the 50 temperature within the chamber is too high, we decrease the amount of external heat insulation, and when the temperature is too low, we increase the amount of this external heat insulation. This external heat insulation 55 may advantageously consist of a layer of dust coal, or other appropriate heat insulating material, loosely packed around the outside of the condenser. The amount of external heat insulation about the condenser is then varied 60 by varying the thickness of this layer of heat insulating material.

The size and proportions of the condenser are varied in accordance with the amount of zinc vapor to be condensed. Working with a 65 retort (10) 8 inches in internal diameter and

10 feet long, charged with zinc silicate ore (containing approximately 45-50% zinc) and dust coal in about equal amounts, and working off the charge in 8 hours, we have secured excellent results with a condenser 70 built of a mixture of carborundum and fire-clay, approximately 12 inches in internal diameter and 11 inches high (internal), the walls of the condenser being 1 inch in thickness. The nozzle 28 was approximately 3 75 inches in internal diameter and extended about 4 inches within the condensing chamber. The exterior of the condenser was covered with about 2 inches of dust coal, as 80 the heat insulating material.

The condenser of Fig. 4 is of the same general type and dimensions as the condenser hereinbefore described in conjunction with Fig. 1. The nozzle 28' of the condenser shown in Fig. 4 is of larger internal diameter than the nozzle 28, and is conical in section. This larger diameter of nozzle 28 permits charging of the retort through the condenser, the charge being introduced through the opening 30 and into the top of the retort 90 through the nozzle 28'. Too large a nozzle, however, is not desirable, since a certain amount of the condensed zinc drops off the ceiling 26, and if the diameter of the nozzle 28' is too large, an objectionable amount of molten zinc drops back into the retort and has to be redistilled.

The condenser of Fig. 5 is relatively higher and narrower than the condensers of Figs. 1 and 4. Care must be taken not to unduly lengthen the condenser, since under such circumstances the top of the condensing chamber becomes relatively cool and an excessive amount of "blue powder" may be formed. In the condenser of Fig. 5 the same reference characters have been used to designate corresponding or equivalent parts as in Fig. 1.

While we prefer to arrange the entrance nozzle or orifice of the condenser so that it is coaxial with the condensing chamber, such an arrangement is not necessary. In Fig. 6 the nozzle 28" for conveying the zinc vapor to the condensing chamber is disposed at one side of the chamber.

The condenser of Fig. 7 is provided with 115 spaced walls. The exhaust gases from the condensing chamber pass through the space between the two walls and thus promote the heat insulation of the condensing chamber. Corresponding or equivalent parts of the condenser of Fig. 7 are indicated by the same reference characters as in Fig. 1. The condenser proper (25-26) is surrounded by a 120 spaced shell 33, of fire-clay or the like. The gases escape from the condensing chamber through openings or ports 35 in the cylinder 25. The gases then flow through the space between the shell 33 and the condenser (25-26) and escape to the atmosphere 125 130

through appropriately positioned openings or ports 34 in the shell.

In the condenser shown in Fig. 8, the upright condensing wall 25' is inclined instead of being vertical. The condenser shown in this figure is thus generally conical in shape. In other respects this condenser is in principle substantially the same as already described.

10 In Fig. 9 of the drawings, we have illustrated a multiple condenser adapted to be used with a vertical retort or shaft furnace of relatively large diameter. As illustrated in Fig. 9, this condenser consists of three or 15 more units, and embodies the general structural features of the condensers of Figs. 1 and 7.

The condensers herein illustrated and described are generally of circular section. 20 However, it is to be understood that this configuration is not an essential part of the invention, but is adopted in practice principally because of its practical convenience. The improved condenser of our invention may be 25 square, rectangular, oval and indeed of any desired, sectional configuration.

The improved condenser of our invention is principally characterized by its upright and preferably vertical condensing wall (or 30 walls) and substantially horizontal ceiling. The condensing surface or area of the upright wall (or walls) and ceiling are carefully proportioned with respect to the amount of zinc vapor to be condensed in a unit of 35 time and this condensing surface is held at a carefully controlled temperature. The current or stream of entering zinc vapor is conducted into the condensing chamber through an opening, preferably constricted, in the 40 bottom of the condenser, and rising upwardly impinges against the ceiling and is deflected over the condensing surface. The zinc vapor repeatedly circulates over the condensing surface, covered with a film of molten zinc, until 45 condensed. The exhaust gas is preferably permitted to escape through the loosely covered opening in the top of the condenser. However, if desired, the upright wall of the condenser may be provided with suitable 50 openings or ports for the escape of the exhaust gas.

The zinc vapor enters the condensing chamber at an approximately right angle to the surface of the molten zinc in the collecting well. The molten zinc in this well preferably surrounds the conduit through which the zinc vapor passes on its way into the condensing chamber. The temperature of the molten zinc in the collecting well is controlled 55 to prevent boiling of the molten zinc. This may be conveniently accomplished by appropriate control of the amount of external heat insulation about this portion of the condenser. The upright wall or walls of the condenser 60 are preferably equidistant from the entering

stream of zinc vapor at any point taken on a horizontal plane through such stream.

As applied to the vertical retort furnace illustrated in the accompanying drawings, the stream of zinc vapor flows upwardly 70 (vertically) from the retort into the condensing chamber, thus making the travel of the vapor in a continuous straight line. This secures the operation with a minimum of back pressure and under natural draft. 75

Assuming that a substantially pure mixture of carbon monoxide gas and zinc vapor issue from the top of the vertical retort 10, the two factors that play a great part in the efficiency of condensation are the temperature and pressure within the condensing chamber. Both of these factors are controlled by the size and the proportions of the condenser. If the temperature of the condensing walls is too great, zinc vapor will 80 escape and be lost. If the temperature is too low, the zinc will condense in the form of "blue powder," rather than molten metal. If the pressure in the condensing chamber becomes too great, it will have a deadening effect on the velocity of the reaction within the vertical retort, and will, therefore, adversely affect the recoveries. If the pressure in the condensing chamber becomes too low, the zinc will condense as "blue powder," 85 rather than molten metal. 90

In operating a zinc distillation muffle or retort on batch charging, rather than continuous charging, the matter of condensation of the zinc vapor becomes more difficult. 100 With continuous charging the ratio of zinc vapor and carbon monoxide gas and the amount of zinc vapor may be held fairly constant and uniform, and a condenser of appropriate size and proportions may be provided for this uniform set of conditions. 105

In the case of batch or intermittent charging, however, considering an eight-hour period to represent one batch or operation, the greater portion of zinc is liberated from the charge in the first four hours of the operation. In addition, in the first four hours of the operation the percentage of zinc in the mixed gases passing from the muffle or retort is less than in the second four hours of the operation. During the first four hours of the operation, the condenser, therefore, should have a relatively large radiating surface and relatively large volume in order to keep the temperature and pressure down to within the limits for efficient condensation. During the latter four hours of the operation, the ratio of zinc in the gases increases and the quantity decreases so that it is necessary to provide more external heat insulation for the condenser in order to maintain a high enough temperature for efficient condensation. It is impossible to change the volume of the condensing chamber and, therefore, during this latter stage of the op- 110 115 120 125 130

eration the pressure in the condensing chamber is too low for efficient condensation, and some of the zinc may, therefore, be condensed as "blue powder."

5 In constructing a condenser for batch or intermittent operation, it is preferable to compromise between the two extreme conditions, rather than to provide a condenser of appropriate size and proportions for one or 10 the other extreme conditions.

We claim:—

1. A condenser for metallic vapors comprising a substantially upright enclosing wall, a ceiling for said wall having an opening therein, a plate loosely covering said opening, and a closure at the bottom of said wall having an opening for the passage of metallic vapor into the condenser.

15 2. A condenser for metallic vapors comprising a substantially upright enclosing wall, a ceiling for said wall having an opening therein, a plate loosely covering said opening, an external covering of heat-insulating material for said wall and ceiling, and 25 a closure at the bottom of said wall having an opening for the passage of metallic vapor into the condenser.

3. A condenser for metallic vapors comprising a substantially upright enclosing 30 wall, a ceiling for said wall, an external covering of loosely packed granular heat-insulating material for said wall and ceiling, and a closure at the bottom of said wall having an opening for the passage of metallic vapor 35 into the condenser.

4. A condenser for metallic vapors comprising a substantially upright enclosing wall, a ceiling for said wall having an opening therein, a plate loosely covering said 40 opening, an external covering of loosely packed granular heat-insulating material for said wall and ceiling, and a closure at the bottom of said wall having an opening for the passage of metallic vapor into the condenser.

45 5. A condenser for metallic vapors comprising a vertically disposed cylindrical enclosing wall, a ceiling for said wall having an opening therein, a plate loosely covering said 50 opening, an external covering of heat insulating material for said wall and ceiling, a closure at the bottom of said wall having an opening therein, and a nozzle extending upwardly from said opening into the condenser.

60 6. A condenser for metallic vapors comprising a vertically disposed cylindrical enclosing wall, a ceiling for said wall having an opening therein, a plate loosely covering said opening, an external covering of loosely packed granular heat-insulating material for said wall and ceiling, a closure at the bottom of said wall having an opening therein 65 and a constricted nozzle extending upwardly

from said last mentioned opening into the condenser.

In testimony whereof we affix our signatures.

GEORGE T. MAHLER. 70  
ERWIN C. HANDWERK.  
EARL H. BUNCE.

75

80

85

90

95

100

105

110

115

120

125

130